

## UNITED STATES PATENT OFFICE.

CHAUNCEY C. LOOMIS, OF YONKERS, NEW YORK, AND HENRY W. BANKS, 3D, OF NOROTON, CONNECTICUT, ASSIGNEES TO THE HEVEA CORPORATION, OF NEW YORK, N. Y.

## FOOTWEAR.

No Drawing.

Application filed May 10, 1924. Serial No. 712,436.

This invention relates to footwear, and has for its object to provide a practical way to sole or re-sole shoes or the like, with a leather substitute which exhibits water-resistant qualities equal to or greater than those of leather; which possesses the unique quality of being attachable to the shoe without sewing or nailing, and which, consequently, can be utilized by the average person unskilled in the shoemaker's trade.

The invention comprehends a method of producing a shoe or similar article of footwear, carrying the new sole characterized in the preceding paragraph, and includes also the completed article that results from the practice of the method.

An illustrative description of the invention is as follows. We may begin with a shoe that is substantially complete, except that it is minus an outsole. In such case the insole will ordinarily be somewhat roughened (at least it will not be too smooth for the purposes of my invention) on its outer surface. If it should happen that it is too smooth, it may be slightly roughened by scoring or abrading, in any suitable way. The invention is, however, equally applicable to worn shoes, for instance, a shoe whose outsole has been worn through at one or more places. In such case the out-sole may be removed, or it may be left in place and suitably roughened for the attachment of the repair or restoration sole as hereinafter set forth.

The repair or substitute out-sole may be produced by providing an aqueous emulsion of rubber, or a quantity of rubber latex, suitably compounded with a dry mix including say 80% of fibrous asbestos and 20% of desired pigment. 65 parts by weight of the dry mix are brought together with sufficient of the emulsion or latex to approximate, say, 35 parts by weight of dry rubber.

We prefer to add also a small amount of sodium silicate, and, if desired, sulphur and an ultra catalyst.

The composition of matter made up as

above suggested, should have the consistency of cream cheese, and in use is merely spread on the leather surface to the desired thickness, the edges of the layer trimmed, and the shoe left in a suitable place until the layer has set sufficiently and proper adhesion thereof to the leather surface has been accomplished. Thereupon, the shoe may be worn, and it will be found that the out-sole will give excellent wear.

We consider that one of the important features of the composition which we employ and which adapts it particularly for use with sole leather, is the use of the aqueous emulsion of rubber, or the rubber latex. This we believe is one of the reasons why we are enabled to apply a single thick layer, which in its subsequent coagulation or setting in situ becomes a homogeneous coherent mass, unusually adhesive with respect to the leather surface. The extraordinary adhesive quality we believe to be at least in part due to the presence of water in the emulsion or in the latex, which possibly facilitates penetration of the leather by the rubber particles held in suspension.

The reason for the presence of a filler, such as asbestos, is of course obvious. This added filler, however, makes it necessary to provide in some way for substantially preventing coagulation of the composition until such time as it is to be actually used. Latex as it is transported in bulk is ordinarily treated with ammonia, which has the effect of preserving the natural protective colloids. However when a considerable body of a foreign substance like asbestos is added to the latex, there is a new condition. Much of the water of the latex is taken up by the asbestos, and the integrity of the natural protective colloids is impaired, if not destroyed. Therefore, we conceived the idea of supplying additional protective colloid content, so that the composition, which is the basis of our invention, may be shipped and handled in bulk substantially without danger of deterioration, especially in so far

as the matter of coagulation is concerned. And we selected as the added protective colloid, sodium silicate, for the reason that we believed (and the results seem to justify the belief) that sodium silicate not only functions as a protective colloid, but increases the adhesiveness of the composition to a leather sole, and possibly also makes for additional coherence in the mass. It is 10 of course well known that sodium silicate is an excellent adhesive, and we have thought that a composition made as above described, except that it was minus the sodium silicate, might be applied to the shoe 15 sole by placing on the sole a layer of sodium silicate, and on that a layer of the composition. This however does not seem to give the best results, possibly because the silicate does not penetrate the leather so 20 well as the water does, and presents a substantial barrier between the openings of the leather and the rubber particles which, for the best results, should be entered into the openings of the leather. Very likely it is 25 a fact that by mixing the sodium silicate through the mass of the composition we effect a compromise, and obtain to a considerable degree the penetrative qualities of the water and the adhesive qualities of the 30 sodium silicate, while incidentally securing the protective effects of the silicate. There is possibly an additional advantage in that sodium silicate is non-organic, and therefore perhaps the less subject to decomposition 35 or chemical change harmful to the mass. Furthermore, though the silicate is water soluble, this does not affect the penetration of the leather to an injurious extent, while of course the mass of the layer insures the 40 retention of the silicate, with its adhesive effects, within the mass and especially as regards its binding effect on the filler.

The suggested addition of vulcanizing agents may be omitted, though a partial 45 cure of the sole may in some cases be desirable.

It is to be understood that the foregoing description, involving particular materials, proportions, and sequences of operations, is 50 merely illustrative, and that no limitations upon the scope of the claims are intended thereby, except such as are properly deducible from the language of the appended claims.

We claim:

1. In combination, a shoe sole, and a supplemental sole adhesively joined thereto, comprising a layer of a composition including an aqueous emulsion of rubber intimately mixed with a filler, said layer being in direct contact with the sole and having a merged-surface relation therewith.
2. In combination, a shoe sole, and a supplemental sole adhesively joined thereto, comprising a layer of a composition includ-

ing an aqueous emulsion of rubber with a filler and an added protective colloid, all intimately mixed, said layer being in direct contact with the sole and having a merged-surface relation therewith.

3. In combination, a shoe sole, and a supplemental sole adhesively joined thereto, comprising a layer of a composition including an aqueous emulsion of rubber with a filler and an added protective-colloid-adhesive, all intimately mixed, said layer being in direct contact with the sole and having a merged-surface relation therewith.

4. In combination, a shoe sole, and a supplemental sole adhesively joined thereto, comprising a layer of a composition including an aqueous emulsion of rubber with a filler and an added non-organic protective colloid, all intimately mixed, said layer being in direct contact with the sole and having a merged-surface relation therewith.

5. In combination, a shoe sole, and a supplemental sole adhesively joined thereto, comprising a layer of a composition including an aqueous emulsion of rubber with a filler and sodium silicate, all intimately mixed, said layer being in direct contact with the sole and having a merged-surface relation therewith.

6. In combination, a shoe sole, and a supplemental sole adhesively joined thereto, comprising a layer of a composition including an aqueous emulsion of rubber with a filler and a pigment, all intimately mixed, said layer being in direct contact with the sole and having a merged-surface relation therewith.

7. In combination, a shoe sole, and a supplemental sole adhesively joined thereto, comprising a layer of a composition including an aqueous emulsion of rubber with a filler and a vulcanizing agent, all intimately mixed, said layer being in direct contact with the sole and having a merged-surface relation therewith.

8. The method of outsoling a shoe which comprises applying to the sole of the shoe a layer of a composition that includes a rubber emulsion and a filler, all intimately mixed, and allowing coagulation of the emulsion to take place in situ, with consequent adhesion of the layer to the sole.

9. The method of outsoling a shoe which comprises applying to the sole of the shoe a layer of a composition that includes a rubber emulsion, a filler, and a protective colloid, all intimately mixed, and allowing coagulation of the emulsion to take place in situ, with consequent adhesion of the layer to the sole.

10. The method of outsoling a shoe which comprises applying to the sole of the shoe a layer of a composition that includes a rubber emulsion, a filler, and a non-organic protective colloid, all intimately mixed and al-

lowing coagulation of the emulsion to take place in situ, with consequent adhesion of the layer to the sole.

agulation of the emulsion to take place in situ, with consequent adhesion of the layer <sup>10</sup> to the sole.

11. The method of outsoling a shoe which comprises applying to the sole of the shoe, a layer of a composition that includes a rubber emulsion, a filler, and sodium silicate, all intimately mixed, and allowing co-

In testimony whereof we affix our signatures.

HENRY W. BANKS, 3d.  
CHAUNCEY C. LOOMIS.